

## UNITED STATES PATENT OFFICE

2,033,885

IMPREGNATING PITCH AND PROCESS AND  
PRODUCT UTILIZING ITIra H. Derby, Indianapolis, Ind., assignor to  
Peter C. Reilly, Indianapolis, Ind.No Drawing. Application December 18, 1931,  
Serial No. 581,987

3 Claims. (Cl. 91—68)

My invention relates to the impregnation of 5  
cellulosic fibrous material and products, such as  
paper, cloth, wood-pulp sheets and conduit, roofing  
paper, and fibrous insulating materials, as  
well as wood itself, with water-proofing com-  
pounds of pitchy character, such as coal-tar pitch,  
water-gas-tar pitch, and/or petroleum pitch,  
and various mixtures of pitches; to the process  
of impregnation involved; to the special impreg-  
nating materials used; and to the final impreg-  
nated materials, more especially impregnated  
conduit.

It is the object of my invention to increase the  
absorption of such pitchy material into the fibrous  
materials to be impregnated, so that a greater  
amount of the pitchy material may be taken into  
the pores of the fibrous material; to serve the  
multiple purpose of increasing the water-imperviousness,  
of increasing both the dielectric strength  
and the mechanical strength, of decreasing the  
lowering of dielectric strength under water-absorption  
conditions, and of improving the appearance  
of the treated material.

This invention is based on the discovery that  
the absorption of pitch by cellulosic fibrous ma-  
terials may be markedly increased in rate and ex-  
tent, and water-imperviousness promoted, by  
the conjoint use with the pitch to be absorbed of  
phenolic tar-acid. By phenolic tar-acid I mean  
such phenolic bodies as those which normally oc-  
cur in coal-tar, and their analogs, homologs, and  
isomerides, whether of synthetic or other origin.  
That is, the tar-acids which I use in any particu-  
lar case may actually be derived from other  
sources than coal-tar.

Among the phenolic tar-acids which are suit-  
able, either in the crude or the refined state, are  
the following:

1. Phenol
2. Various composite tar-acids (from tar-acid oil)
3. Various cresylic acids
4. Ortho-cresol
5. Para-cresol
6. Meta-cresol
7. Mixtures of cresols, as of meta-cresol and  
para-cresol
8. Xylenols
9. High-boiling tar-acids
10. Low-temperature tar-acids
11. Ortho-phenyl-phenol
12. Alpha-naphthol
13. Beta-naphthol
14. Pyro-cresols
15. Various mixtures of the preceding phenolic  
tar-acids
16. Mixtures of oils with the tar-acids or with  
mixtures of tar-acids, whether the oil is  
a tar oil or some other kind of oil such  
as petroleum oil.

In carrying out my invention I may use any  
suitable impregnating pitch; and I use with it a  
phenolic tar-acid material such as referred to  
above. The pitch I prefer is a water-gas-tar  
pitch which melts between 50° and 80° C. The 5  
additional material may be mixed with the pitch,  
and the mixture applied as a unit in a single  
impregnating process; or the additional ma-  
terial may be preliminarily applied to the fibrous  
material to be impregnated, and the pitchy ma-  
terial applied subsequently. The temperature  
used for impregnation should be sufficiently high  
to make the impregnating materials flow fairly  
freely, and should be as high as conveniently pos-  
sible without causing deterioration of either the 15  
treated or the treating materials. In practice,  
the impregnating temperature is well over 100°  
C., but usually under 200° C.; and for most  
pitches a satisfactory impregnating temperature  
is about 160° to 170° C. The impregnation may 20  
be made by simply soaking the fibrous material  
for a suitable time, or may be made under pres-  
sure to obtain greater penetration in shortened  
time.

I will describe my invention particularly with 25  
reference to the impregnation of electric con-  
duits, of the type made of news-print paper-pulp  
or wood-pulp; and from that it will be clearly ap-  
parent how my invention is used on other types  
of cellulosic fibrous material.

These conduits are commonly from about 2 to 8  
inches across, in length of from 3 to 12 feet, with  
walls of from  $\frac{1}{8}$  inch to  $\frac{3}{4}$  inch in thickness, or  
thereabouts. After being formed, these conduits  
are desirably dried before impregnation.

For many years it has been the custom to im-  
pregnate these conduits with pitch, by immersing  
them in a pitch bath for 7 or 8 hours and then  
allowing them to cool, with the pitch bath main-  
tained at a temperature of about 150° to 185° C. 40  
The normal mean absorption of pitch has been  
in the neighborhood of 140% to 180% of the  
weight of the untreated conduit. A conduit so  
treated is fairly water-impervious, but not so  
much so as is to be desired. When tested for 45  
water absorption by being immersed in water at  
21° C. for 48 hours the mean absorption of water  
is ordinarily found to be from 5% to 15% of the  
weight of the pitch-treated conduit. When such  
absorption of water occurs in a conduit in actual  
use, the resultant lowering of dielectric strength  
is very pronounced, amounting ordinarily to  
about 40% to 60%.

Instead of using the simple pitch that has  
heretofore been used for impregnation, I use 55  
such pitch together with some one or more of  
the phenolic tar-acids above referred to as the  
impregnating material. The quantity of tar-  
acid used may be relatively small in comparison  
to the quantity of pitch. In most instances it is

- sufficient to use as little as from 1% to 3% tar-acid as reckoned on the weight of the pitch used; although in some instances it is desirable to use more tar-acid than that for best results, up to 5 8% or 10% in the case of beta-naphthol for instance, while in others it is possible to get good results with less, for instance as little as 0.2% in the case of crude composite tar-acids from tar-acid oil. In any case, it is desirable to use enough 10 of the phenolic tar-acid to cause an increase in the total quantity of pitch which will be absorbed by the cellulosic fibrous material (the conduit) in a given time under specified conditions.
- 15 It is found that with conduit thus impregnated, so that a greater amount of pitch is absorbed, the water-imperviousness of the conduit is markedly increased over that of previously known conduits, the proportionate increase varying 20 with the nature and amount of the tar-acids used. The pitch absorption by the use of the tar-acids may be increased by as much as 40% or 50% in some instances, over that of the unmodified pitch; and the mean water absorption of 25 the conduit so impregnated with the modified pitch under the test for absorption by immersion in water for 48 hours at 21° C., may easily be reduced to below 3% of the weight of the treated conduit, and in most cases below 1% thereof.
- 30 In many instances, with this water-absorption test, we have been able to get a mean absorption below 0.5% of the weight of the treated conduit. Thus the lowering of water-absorption under given conditions is of the order of 40% to 90%, 35 and even more in some instances, as compared to previous commercial pitch-treated conduits.
- The following table shows some results that were actually obtained by the use of water-gas-tar pitch melting between 50° C. and 80° C. and 40 containing the indicated percentages of various phenolic tar-acids.

| 45 | The material added to the pitch                         | Percentage absorption of treating material | Percentage water absorption in 48 hours at 21° C. |
|----|---------------------------------------------------------|--------------------------------------------|---------------------------------------------------|
|    |                                                         | Percent                                    | Percent                                           |
| 50 | 0.5% crude composite tar-acids.....                     | 228                                        | 0.32                                              |
|    | 1.0% crude composite tar-acids.....                     | 251                                        | 0.27                                              |
|    | 2.0% crude composite tar-acids.....                     | 271                                        | 0.15                                              |
| 55 | 2.0% ortho-cresol.....                                  | 223                                        | 0.24                                              |
|    | 2.0% para-cresol.....                                   | 226                                        | 0.40                                              |
|    | 2.0% high-boiling tar-acids.....                        | 246                                        | 0.23                                              |
|    | 2.0% light-oil and tar-acid mixture.....                | 242                                        | 0.09                                              |
|    | 2.0% alpha-naphthol.....                                | 248                                        | 0.08                                              |
|    | 4.0% phenol.....                                        | 228                                        | 0.7                                               |
| 60 | 2.0% crude composite tar-acids (4½ hour treatment)..... | 263                                        | 0.12                                              |
|    | 2.0% crude composite tar-acids (1 hour treatment).....  | 194                                        | 1.1                                               |

60 The treatments shown in the above table, except the last two, were all for 7½ hours, the first 7 hours at 160° C. and the last ¾ hour at 182° C.; which conforms to standard practice in impregnating conduits. The last two lines of the 65 table, however, show that in my process it is possible to use a shortened treatment, for there the treatments were for totals of only 4½ hours and 1 hour respectively, at 160° C.

70 Thus a marked increase in the amount of pitch absorbed, and/or a great saving in impregnating time, may be obtained in impregnating processes by the use of my modified pitch. The saving in impregnating time is especially marked when the impregnation is carried only to the extent of previous impregnations.

In the examples shown in the table given above the treatment is made by mixing the pitch and the indicated phenolic tar-acid, and impregnating the conduit in a single impregnating treatment. However, I have also gotten good results 5 by treating the conduit first with the phenolic tar-acid and subsequently impregnating with the pitch. In the latter case, the treatment of the conduit with the tar-acid may be in any convenient way, as by dipping, brushing, or spraying, 10 using either the tar-acid alone, the tar-acid dissolved in a solvent (such as benzol), or the tar-acid made into an emulsion (even with water). The amount of tar-acid used is so small in comparison to the pitch that when it is applied 15 preliminarily it is not in sufficient amount to make a complete impregnation by itself of the treated material; but it somehow combines with and modifies the subsequently applied pitch so that the penetration of the latter is facilitated. 20

With the impregnation by modified pitch as above outlined, I not only get an increase in the amount of absorption of the treating material, and a decreased amount of water-absorption under similar water-exposure conditions, but I 25 also get an increase in the dielectric strength of the conduit, an increased mechanical strength, a decrease in the proportionate lowering in dielectric strength under given water-exposure conditions, and an improved appearance. The surface 30 of the conduit which has been treated with my modified pitch is usually a uniform lustrous black on both inner and outer surfaces, with a thin but even outer seal coating instead of the thick irregular outer coating seen in those previous conduits in which it has been sought to obtain a seal coat. If preferred, a dull surface may be obtained, for instance if phenol or meta-cresol is used as the pitch-modifying agent. 35

Although I have primarily described my invention 40 for electric conduit, in which telephone or telegraph or similar conductors are placed, my invention is applicable to various other cellulosic fibrous materials. For instance, fabric insulation can be impregnated in the manner described 45 above for conduit. So can wood; although it is desirable to dry the wood first, so that penetration into the wood may not be interfered with by moisture in the wood-pores. The wood that is treated may have been previously creosoted if desired. I have also used the same impregnating 50 materials and processes for vegetable-fiber plates or sheets, such as various wall-boards, fibrous-base tiles, etc. These are merely examples of the materials to which my invention is applicable. 55

I claim as my invention:

1. The process of treating relatively inflexible prefabricated cellulosic fibrous material, which consists in impregnating it with water-gas-tar pitch containing from 0.2% to 10.0% of phenolic tar-acid.

2. An impregnating pitch of the class consisting of coal-tar pitch and water-gas-tar pitch, containing between 0.2% and 10.0% phenolic tar-acid, for impregnating relatively inflexible prefabricated cellulosic fibrous material such as conduit.

3. An impregnating pitch comprising water-gas-tar pitch melting between 50° and 80° C., to which has been added phenolic tar-acid, for impregnating relatively inflexible prefabricated cellulosic fibrous material such as conduit.